

## UNITED STATES PATENT OFFICE

2,120,851

PROCESS FOR THE MANUFACTURE OF  
SPUN GOODS, FABRICS, AND OTHER  
TEXTILESOskar Walter Becker and Hans Freudenberg,  
Weinheim, Germany, assignors to Carl Freud-  
enberg G. m. b. H., Weinheim, Germany, a Ger-  
man companyNo Drawing. Application September 9, 1935,  
Serial No. 39,864. In Germany September 19,  
1934

## 14 Claims. (Cl. 18—54)

This invention relates to a process for the manufacture of spun goods, fabrics and other textiles, with the employment or co-employment of threads obtained from animal hide material.

5 According to this invention it has been found that textiles as aforesaid can be manufactured with the employment of threads, which have been obtained by converting the hide material with the aid of swelling agents and, if desired, by mechanical treatment, into a pasty slippery condition whilst maintaining the fibres and thereafter extruding the paste under high pressure through tapering nozzles.

10 It was contrary to all expectation that it would be possible directly to obtain threads, adapted to be spun and woven and subjected to other textile operations, merely by converting the skin or hide into a paste and extruding this paste under high pressure through tapering nozzles.

15 20 The treatment of the hide material with swelling agents and any mechanical treatment must be continued until a fibre-containing paste of slippery consistency is obtained, in which the absorbed water is fixed as swelling water, i. e. is incapable of being expressed even under the application of pressure, and in which the individual fibres can readily slide over one another. Threads of the diameter customarily employed in the manufacture of textiles can only be produced 25 from a paste of the aforesaid consistency by direct extrusion through nozzles.

25 30 The process of this invention is carried into effect by causing the hide material to undergo extensive swelling either in an alkaline or an acid medium. A treatment with alkaline liquids may also be followed by a treatment with acid liquids. The treatment is preferably not carried out in the neighbourhood of the isoelectric point, but either in a pronounced alkaline medium at pH values over 12, or in a pronounced acid medium at pH values below 4. The skin or hide may for example be subjected to prolonged liming and be thereafter treated with acids, particularly hydrochloric acid. Other acids, such as formic acid or 35 40 45 50 lactic acid, may be employed instead of hydrochloric acid. The swelling treatment may also be carried out exclusively in an alkaline medium, for example in milk of lime or dilute caustic soda solution or successively in both.

50 The swelling treatment may be promoted by mechanical treatments, such as comminuting, pounding, pressing and the like. It is finally advisable to homogenize the fibrous paste by treating the same in a kneading machine or mixer,

whereby the fibrous pulp may also be adjusted to the desired water content.

5 In general it is advisable to prepare a fibrous hide paste, which contains at least 80% of water in order to enable technically obtainable pressures to be employed for extruding the paste through nozzles. It is advisable to adjust the fibrous hide paste to a content of 6 to 12% of dry substance. Satisfactory results have, however, also been obtained with masses having a still lower content of dry substance.

10 The fibrous hide paste prepared as aforesaid is extruded under high pressure through nozzles. Constantly and gradually tapering long nozzles may be used, in which event the fibrous hide mass acquires only a relatively slight acceleration during extrusion. Nozzles, which taper considerably along a relatively small length may, however, also be used. The diameter of the discharge opening of the nozzles should in 15 general amount to from 0.01 to 0.5 mm. Nozzles of smaller or greater diameter may also be used, depending on the thickness of thread required in the further working up thereof into textiles. The characteristic feature of this invention is 20 that the threads required for the further working up into textiles are obtained by extruding the fibrous hide mass through the nozzles directly, i. e. without subsequent further comminution or shredding.

25 30 35 In the further development of this invention it has been found that textiles can be manufactured with the employment of short threads, which have been obtained by effecting the production of the threads from the fibrous hide paste, for example the extrusion through nozzles, or the further working up of the filaments, for example the withdrawal thereof, under such conditions that the artificial threads are divided into short pieces.

40 45 50 The production of the short threads is for example effected by employing a periodically changing pressure when extruding the fibrous hide paste through tapering nozzles. Short threads may, however, also be obtained by extruding the paste through the nozzles under uniform pressure and taking up the long threads discharging from the nozzle on belts, which move intermittently or in jerks and thereby tear the threads into small pieces. The long threads may, however, also be torn or cut into small pieces at any other stage of the production, for example after drying or tanning. The resulting short threads may be of varying lengths depending on the adjustment of the mechanical conditions. In 55

general the operation is carried out in such a way as to produce short threads 3 to 5 cms. in length.

The thread discharging from the nozzle may be dried in a manner known per se, the colloid substance contained in the paste causing the surface of the thread to be sized. The sized thread can be rendered waterproof by treatment with tanning agents. An alternative procedure is directly to tan the threads discharging from the nozzles, for example by intercepting the threads in a suitable tanning bath. A second alternative is to size the threads, obtained by extrusion through nozzles and torn into short pieces by being taken up on an intermittently moving belt, by drying them on this belt or to tan them by spraying with tanning liquids. A third alternative is to cause the discharging threads to be taken up on belts, particularly intermittently moving belts, which pass beneath tanning liquids.

In many cases it is advisable to twist the threads discharging from the nozzles before or during the sizing operation. Several threads may also be twisted together. It is sometimes advisable again to render the already sized threads sticky and only thereafter to twist the individual threads or bunches of threads. In this event the threads may be rendered waterproof with the aid of tanning agents before, during or after the twisting operation.

The threads may also be treated in the course of their production with agents which are adapted to improve their properties. Examples of agents as aforesaid are those which are capable of diminishing or removing the hydrophilic properties of the threads or of altering and improving the threads with regard to elasticity, pliability, crimping, lustre or colour. Examples of agents adapted to improve the properties of the threads are softeners, wetting agents, mordants, fats, colours and the like.

The resulting threads may be worked up alone or in conjunction with other fibres by the methods usually employed in the textile industry.

45

#### Examples

1. Neats' hides after a liming treatment of about four weeks are washed and brought by swelling with hydrochloric acid to a dry substance content of 12%. The hide material is then resolved with the aid of rollers and the fibrous mass is homogenized by kneading with water and adjusted to a dry content of 5%. This mass is extruded under a pressure of 500 atms. through tapering nozzles. The thread discharging from the nozzle is dried in the air, whereby it becomes sized on the surface by the setting of the colloidal substances contained therein, and rinsed. The thread is rendered waterproof by alternately moistening three times with a hardening liquid obtained from the distillation of wood and three times drying, and can thereafter be again rendered soft, lubricated and coloured.

2. Pigs' skins, after removing the fat, are de-haired by liming, limed for eight days, then washed and acidified with hydrochloric acid. The resulting fibrous hide paste is extruded through nozzles as described in Example 1. The resulting threads are rendered waterproof by treatment in chromium sulphate baths.

3. Calves' skins of inferior quality after de-hairing are limed for six weeks, rinsed and resolved by extruding through nozzles of 2 mms. diameter. The resulting cords of fibrous mass 75 are kneaded with 0.1% caustic soda solution,

brought to a water content of 90% and then extruded through nozzles and further treated as described in Example 1.

4. Shark skin is washed in cold water, thereafter de-fatted in acetone, softened and freed from scales by one of the usual processes, thereafter limed for four weeks, partially freed from lime by washing and crushed between crushing rollers whilst still in a lime-swollen condition. The loosened skin is disintegrated in a Hollander into a fine fibrous material and rendered iso-electric. The excess water is removed by expressing and the resulting fibrous material is adjusted with lactic acid in a kneading apparatus to a pH value of 3.5 and worked up into a homogeneous paste. The fibrous material obtained is extruded through tapering nozzles and the thread further worked up as described in Example 1.

5. De-tanned chrome leather parings are subjected to additional liming for three weeks, thereafter extensively freed from lime in a washing Hollander, then partially freed from water by suction, adjusted to a pH value of 2.4 with hydrochloric acid, thereafter worked up to a homogeneous paste containing 4% of dry substance and extruded through tapering nozzles under a pressure of 100 atms. The thread discharging from the nozzle is dried and conveyed through a chromium sulphate bath containing 7% of Glauber's salt as a protection against swelling, rinsed, thereafter introduced for four weeks into a hot, moist chamber for the purpose of re-tanning, thereafter rinsed, drawn through lubricating and dyeing baths and finally dried under tension.

6. Cattle sinews after two weeks liming are washed with water and swollen with hydrochloric acid. The pH value is adjusted by washing to 2.5 to 3.5 and the swollen sinews are crushed between rollers. The resulting mass is rendered uniform by kneading and extruded through tapering nozzles into a pickle bath containing 7% of common salt. In order to increase its tensile strength the thread is twisted in the pickle bath, thereafter tanned, dried and lubricated.

7. Neats' hides after a liming period of four weeks, are washed, brought to a pH value of 2.8 by the addition of hydrochloric acid and adjusted by the addition of water to a dry content of 12%. The swollen hide material is resolved between rollers and the resulting mass is kneaded with water until it acquires a dry content of 5%. This mass is extruded through continuously tapering nozzles. The threads discharging from the nozzles are taken up on a belt which moves intermittently or in jerks and thereby tears the threads discharging from the nozzles into artificial fibres of 3-5 cms. length, which are then dried on the belt by a current of air and are rendered waterproof by repeated moistening with a hardening liquid obtained from wood distillates.

8. Strips of sharks' skin are laid for six weeks in milk of lime, the lime then removed by washing with flowing water until neutral and swollen in water by the addition of hydrochloric acid until the mass acquires a water content of 90%. The strips are then extruded through nozzles of 5 mms. diameter and the resulting threads thoroughly mixed in a kneading machine. The resulting mass is extruded from continuously tapering nozzles under periodically changing pressure and the resulting threads are intercepted in a hydrochloric acid-common salt pickle. The threads which curl up in this bath are conveyed by means of a perforated belt into 75

5 a chrome tanning bath, where they remain for some time in constant movement. The threads are conveyed from the chrome bath into the air by means of a perforated belt and disposed in a hot moist chamber until completely re-tanned. The threads can then be further lubricated and coloured.

10 9. De-tanned and acidified chrome leather parings are kneaded and the resulting mass is extruded through continuously tapering nozzles. The threads discharging from the nozzles are taken up on an intermittently moving belt and sprayed with a hardening liquid. The threads are thereby torn into artificial fibres of 3-5 cms. 15 length and simultaneously rendered waterproof.

10 10. Cattle sinews, converted by swelling, shredding and kneading with water with the addition of hydrochloric acid into a slippery fibrous paste, are extruded through nozzles under periodically 20 changing pressure and the resulting short threads are intercepted in an ammonium chloride pickle. The resulting threads are screened off, tanned with a 10% sumac solution, stored until completely tanned, washed, dried and thereafter 25 coloured.

11. Pig skins after removing the fat and de-hairing are limed for eight days, then washed and treated with hydrochloric acid until thoroughly swollen. The swollen hide material 30 is shredded between rollers and the fibrous mass is homogenized by kneading and adjusted to a dry content of 4%. This paste is extruded under periodically changing pressure into a hydrochloric acid-common salt pickle, in which the resulting 35 short threads are twisted individually or in bunches of several threads together. The threads are then lubricated and tanned. Alternatively the threads may be directly intercepted in a tanning bath and be twisted during the tanning 40 operation. The twisted threads are subjected to chrome tanning and thereafter stored until completely tanned.

What we claim is:

1. In a process for the manufacture of spun 45 goods, fabrics, and other textiles employing threads obtained from animal hide material, the improvement which comprises converting said hide material into a highly swollen slippery paste which contains at most 20% of dry substance 50 and which is substantially free from expressible water by treatment with swelling agents without substantially destroying the fibres, extruding the resulting fibrous hide paste under high pressure through tapering nozzles to produce said 55 threads, drying said threads and rendering said threads waterproof by treatment with tanning agents.

2. A process according to claim 1, wherein the conversion of the hide material into the pasty 60 slippery condition by treatment with swelling agents is promoted by mechanical treatment.

3. A process according to claim 1, wherein the fibrous hide paste contains 6-12% of dry substance.

65 4. A process according to claim 1, wherein the nozzles employed for the production of the threads have an outlet diameter of 0.01 to 0.5 mm.

5. A process according to claim 1, wherein the extrusion of the fibrous hide paste through the

nozzles is effected under periodically changing pressure.

6. A process according to claim 1, wherein the threads discharging from the nozzles are taken up on intermittently moving belts.

7. A process according to claim 1, wherein the long threads produced by extruding through the nozzles under uniform pressure are divided in the course of their further working up into short threads.

8. A process according to claim 1, wherein the threads discharging from the nozzles are dried and thereby sized on the surface by the setting of the colloidal substances contained therein.

9. A process according to claim 1, wherein the threads discharging from the nozzles are twisted individually or several together and are thereafter dried whereby said threads are sized by the setting of the colloidal substance contained therein.

10 10. A process according to claim 1, wherein the threads discharging from the nozzles are twisted individually or several together and are simultaneously dried whereby said threads are sized by the setting of the colloidal substance contained therein.

11. A process according to claim 1, wherein the threads discharging from the nozzles are dried, twisted and rendered waterproof by treatment 30 with tanning agents.

12. As new articles of manufacture dried and tanned filaments composed of collagenous animal fibres of substantially the same length as those contained in the natural hide embedded in a colloidal protein substance which filaments have 35 been formed by expressing a fibrous paste of animal hide material which contains at most 20% of dry substance and which is substantially free from expressible water and drying the expressed filaments whereby said filaments are sized by the setting of the colloidal substance contained therein.

13. As new articles of manufacture threads composed of twisted dried and tanned filaments composed of collagenous animal fibres of substantially the same length as those contained in the natural hide embedded in a colloidal protein substance which filaments have been formed by expressing a fibrous paste of animal hide material which contains at most 20% of dry substance 45 and which is substantially free from expressible water and drying the expressed filaments whereby said filaments are sized by the setting of the colloidal substance contained therein.

14. Spun goods, fabrics and other textiles composed of dried and tanned filaments composed of collagenous animal fibres of substantially the same length as those contained in the natural hide embedded in a colloidal protein substance which filaments have been formed by expressing 50 a fibrous paste of animal hide material which contains at most 20% of dry substance and which is substantially free from expressible water and drying the expressed filaments whereby said filaments are sized by the setting of the colloidal 55 substance contained therein.

OSKAR WALTER BECKER.  
HANS FREUDENBERG.